

# UNITED STATES PATENT OFFICE.

JOSEPH TURNER AND HARRY DEAN, OF HUDDERSFIELD, ENGLAND, ASSIGNEES TO  
READ HOLLIDAY & SONS, LTD., OF HUDDERSFIELD, ENGLAND.

## DYEING VEGETABLE FIBERS.

1,105,722.

Specification of Letters Patent.

Patented Aug. 4, 1914.

No Drawing.

Application filed March 18, 1913. Serial No. 755,103.

To all whom it may concern:

Be it known that we, JOSEPH TURNER and HARRY DEAN, subjects of King George V of Great Britain, and residents of Huddersfield, in the county of York, England, have invented certain new and useful Improvements in Dyeing Vegetable Fibers, of which the following is a specification:

Our invention relates to a new and useful method for dyeing cotton fibers which have been previously dyed with sulfur colors, and to the new and useful products produced thereby.

We have discovered that cotton which has been dyed with sulfur colors can be after-treated with certain amino compounds, and in such a manner that the produced results have many valuable commercial advantages over the untreated or original dyeings.

Our process, in general, consists in treating cotton dyed with sulfur colors with certain amino compounds in the presence of an oxidizing agent. Among the amino compounds which we have employed for the production of these new and valuable results are: paraphenylenediamin; p-amido-p-oxydiphenylamin; paramidophenol; orthoamidophenol; homologues of the fore-mentioned, and the following condensation products which are described in English Patent No. 15008, 1908, viz: paraphenylenediamin and 1 mol. naphthol; paraphenylenediamin and 2 mols. naphthol; paraphenylenediamin and 1 mol. phenol; paraphenylenediamin and 2 mols. phenol; paraphenylenediamin and 1 or 2 mols. cresol; paraphenylenediamin 1 or 2 mols. metaphenylenediamin. In order to produce varied results the above amino compounds may be used singly or in combination with each other.

One method of following our process is as follows: Cotton which has been dyed with 6% of sulfur color, such as cross dye black B. X. is worked in a bath containing 2% paraphenylenediamin, 20 parts of water,

3% acetic acid (50%), 1% bichromate of soda, for a few minutes in the cold and then gradually raised to 40 C. during about half an hour. The operation may also be conducted in the cold throughout or the temperature may be raised to boiling point.

We do not limit ourselves to the exact proportions given above, all of which may be varied without going beyond the scope of our invention.

The herein described method of treatment produces results possessing decidedly different and more valuable properties than those of the original dyed cotton, among which are their increased intensity and beauty of shade and their improved fastness to light and milling.

Having thus described our invention, what we claim is:

1. The process of treating dyed cotton which comprises subjecting cotton previously dyed with sulfur colors to a bath containing an oxidizing agent and an amino compound.

2. The process of treating dyed cotton which comprises subjecting cotton previously dyed with sulfur colors to an acid bath containing an oxidizing agent and an amino compound.

3. The process of treating dyed cotton which comprises subjecting cotton previously dyed with sulfur colors to a bath containing an oxidizing agent and a mixture of amino compounds.

4. The process of treating dyed cotton which comprises subjecting cotton previously dyed with sulfur colors to an acid bath containing bichromate of soda and an amino compound.

Signed at Huddersfield in the county of York, England March, A. D. 1913.

JOSEPH TURNER.  
HARRY DEAN.

Witnesses:

FREDERICK SYKES BAINES,  
VICTOR H. GOLDSMITH.